

# United States Patent Office

3,153,638

Patented Oct. 20, 1964

1

3,153,638

## PLASTICIZED VINYL POLYMER ORGANOSOL COMPOSITION

Wesley Albion Tarwid, Barrington, Ill., assignor to American Can Company, New York, N.Y., a corporation of New Jersey  
No Drawing. Filed Dec. 21, 1959, Ser. No. 860,711  
11 Claims. (Cl. 260—32.8)

The present invention pertains to a novel organosol coating composition, and in particular it pertains to an organosol coating composition having a relatively high nonvolatile content with a relatively low viscosity.

By nonvolatile content as used herein is meant those ingredients having a very low vapor pressure whereby when once incorporated in the organosol, they are not vaporized to any appreciable extent even at the elevated temperatures at which the organosol is fused into a solid film.

Organosols, as the term is generally understood in the art, are essentially a dispersion of a high molecular weight, insoluble polyvinyl chloride resin in a liquid vehicle comprising a careful balance of dispersant and diluent. Because of the inertness and chemical resistance of the films formed therefrom, organosols have found great utility as protective coatings for various substrates, including sheet metal. However, when formulated to give the maximum protection as a sheet metal coating, organosols have the disadvantage of exhibiting a relatively high viscosity preventing rapid and efficient application to the sheet metal, particularly when individual sheets are coated rather than a continuous web of metal.

In the past, the results of thickness, cohesion and flexibility desired of an organosol have been obtained by various means. Thickness is often obtained by building up the organosol film in layers. The most usual means of obtaining cohesive strength and flexibility is by incorporating lower molecular weight solution resins and chemical plasticizers which practice produces high viscosity organosols. Each of these prior art devices for producing a satisfactory organosol coating for sheet metal, because of the high viscosity of the composition, necessitates multiple passes through the coating apparatus and/or single pass coating methods which are not practicable for coating individual sheets, such as knife coating or reverse roller coating.

In the metal can manufacturing industry, and in many other industries, by far the most usual method of protectively coating individual metal sheets is by single pass, direct roller coating, i.e., the applicator roller and the sheet being coated are traveling in the same direction at their line of contact. The high viscosity prior art organosols are unsuitable for application by the direct roller coating technique, causing the operation to be slow and inefficient and tending to produce a finished coating having unsightly and deleterious ridges. Knife-coating, reverse roller coating, i.e., the applicator roller and the sheet are traveling in opposite directions at their line of contact, and similar methods, compared to direct roller coating, as stated previously, are practicable only for coating continuous webs but not for rapidly coating individual, spaced sheets passed through the coating apparatus in sequence.

To produce the final, coherent protective film, the wet organosol coating must be fused by heating to a temperature in the range of about 350° F. to 400° F. This necessity gives rise to another disadvantage of prior art organosols in that the plasticizers used tend to evolve an undesirable amount of obnoxious smoke during the fusing or baking operation.

It is, therefore, an object of the present invention to provide a fluid organosol coating composition which con-

2

tains sufficient film forming nonvolatiles to produce a highly inert, corrosion resistant, ridge-free coating for sheet metal while at the same time having a sufficiently low viscosity at application temperatures so that the organosol can be efficiently applied by direct roller coating.

A further object is to provide a fluid organosol coating which can be applied with equal facility to both a moving, continuous web of sheet metal and to individual sheets of sheet metal passing through the coating apparatus in rapid succession.

Another object is to provide a composition of the character described that contains only a minimal amount of liquid ingredients that adversely affect the polyvinyl chloride dispersion resin.

Still another object is to provide a fluid organosol coating composition for sheet metal which, upon the fusing or baking thereof, knits well to form a continuous, chemically resistant, flexible film which is ridge free and has cohesive strength.

Yet another object is the provision of a composition of the class described which evolves little or no obnoxious smoke during the baking thereof.

Numerous other objects and advantages of the invention will be apparent as it is better understood from the following description which is of a preferred embodiment thereof.

The above and other objects are obtained by using in a fluid organosol coating composition containing a high molecular weight, insoluble vinyl chloride polymer as the dispersion resin, a specific vinyl chloride-vinylidene chloride interpolymer as the solution resin, a polymeric, resinous plasticizer and a careful balance of organic liquids constituting the dispersants and diluents.

The dispersion resin is a vinyl chloride polymer which is relatively insoluble in the dispersants usually used in organosols such as ketones, e.g., acetone, and even to a lesser degree in aromatic and aliphatic hydrocarbon solvents. At most, the polyvinyl chloride dispersion resin must be no more than swelled by the action of ketones utilized as dispersants in organosols. Although aromatic hydrocarbons also have a swelling action on the dispersion resin, their swelling action is not as great as the swelling action of the usual organosol dispersants. Aliphatic hydrocarbons have little or no swelling action on the dispersion resin. The average molecular weight of the dispersion resin must be at least 20,000 and preferably about 20,000. Dispersion resin composed wholly of polyvinyl chloride or copolymers of vinyl chloride with other polymerizable olefinic materials in which copolymer, the combined vinyl chloride content, is greater than 90% are satisfactory. Examples of such copolymerizable olefinic materials are vinyl esters such as vinyl acetate, acrylonitrile and acrylic esters such as methyl and ethyl acrylate or methacrylate, and maleate esters such as dibutyl maleate. The amount of dispersion resin operable is about from 50% to 80% and preferably about 60% to 70% of the nonvolatiles in the organosol.

The primary utility of the organosol coatings of the present invention are as coatings on the inside of metal cans where the organosol is in constant contact with the packed product during the useful life of the can. For this reason, chemical plasticizers, most generally used as dispersants in prior art organosols, cannot be used where good chemical resistance is desired. Aside from the fact that these chemical plasticizer dispersants tend to evolve obnoxious smoke during the fusing of the film, they reduce if not destroy the resistance and inertness of the final coating film to many of the various products packed into the can, especially corrosive products such as strong acids or alkalies, e.g., high pH liquid detergents, by being leached out of the film over a period of time. The dispersant used in the present invention is a low boiling

ketone, or an ether-alcohol or mixture of the two. This dispersant performs the function necessary for an organosol dispersant of forming strong attachments to the dispersion resin, aiding in the wetting of the resin and swelling and softening of the dispersion resin to permit reduction of agglomerates to their basic particles and to give the organosol sufficient viscosity to prevent settling of the particles. In addition, during fusion or baking of the film, the volatile dispersant aids in "knitting" the dispersion resin particles into a continuous film. After having performed its necessary functions, the dispersant is completely and readily removed from the film by the heat of the baking operation without evolution of smoke, leaving behind no undesirable component or residue.

The amount of dispersant in the organosol must be sufficiently high to produce the results stated above but at the same time must not be so high as to cause excessive swelling of the dispersion resin, too great an increase in viscosity and possibly gelation of the organosol. In the instant invention, the range of dispersant content in the organosol must be about from 10% to 50% and preferably about 36% by weight of the volatile liquid constituents of the organosol.

Any aliphatic ketone having a boiling point in the range of 235° F. to 425° F. may be used as the dispersant ketone. Examples of such ketones are diisobutyl ketone, methyl isobutyl ketone, 2,6,8-trimethyl nonanone-4, with diisobutyl ketone being preferred. As an ether-alcohol dispersant there may be used any ether-alcohol having a boiling point in the range of 255° F. to 450° F. To be operable, it is necessary for the dispersant to be of sufficiently high volatility to be removed completely from the organosol during the fusing thereof; but at the same time, to be of sufficiently low volatility to remain in the fluid organosol for as long as possible in order to perform its functions as a dispersant. Specific ether-alcohols useful in the present invention are the 1 to 4 carbon atom alkoxy monoethers of ethylene glycol, such as 2-methoxy ethanol, etc. and diethylene glycol monobutyl ether, with the diethylene glycol monobutyl ether being preferred. If a mixture of ketone and ether-alcohol is used, the weight ratio of ketone to ether-alcohol must be about from 0.05/1 to 1/0.5 and preferably about 0.75/1.

Xylene, toluene, benzene, or similar aromatic hydrocarbons or mixtures thereof are used as the volatile diluent in the organosols of the present invention. Although these aromatic hydrocarbons have a swelling effect on the polyvinyl chloride dispersion resin, they have little or no dispersing action thereon, and therefore cannot be considered as a substitute for or equivalent to the dispersant. In other words, to produce the desired results, the instant organosol can contain only sufficient dispersant to provide a certain amount of dispersion resin swelling and a good dispersion of the resin. The diluent provides the remainder of the volatile liquid necessary to produce additional resin swelling, if needed, proper nonvolatile content and viscosity of the organosol. The aromatic hydrocarbon diluents serve another important function more fully described hereinafter. In the instant invention, the amount of aromatic diluent used is in the range of about from 50% to 90%, and preferably about 64% by weight of the volatile liquid constituents of the organosol, i.e., the combined dispersant and diluent content. The diluent is also smokelessly removed from the composition during fusing.

The solution resin which gives the organosol of the instant invention its unique and novel properties conforms to the schematic formula  $(\text{CH}_2-\text{CH}_{2-n}\text{Cl}_n)_x$  in which  $n$  is either 1 or 2 and  $x$  is a positive number greater than 1. Since, in a given group of chlorethylene units, it is impossible to determine which chlorethylene units have a single chlorine atom and which have two chlorine atoms,  $n$  is said to have an average value of greater than 1 but less than 2 for such a group. Such resins are characterized by being at least 97% completely soluble in liquid ben-

zenoid aromatic hydrocarbons in concentrations up to at least 32% by weight; and their total content of chlorine lies between 61 and 64% by weight.

Specifically, the useful solution resin is composed of thermoplastic chemically saturated polymeric material made up exclusively of carbon, hydrogen and chlorine atoms and comprising recurring units of chlorethylene having from 1 to 2 chlorene atoms on only one of the ethylene carbons and is further characterized by possessing a chlorene content of about 61% to 64% by weight, by having a specific viscosity within the range of about 0.15 to 0.30 as determined at 20° C. using a 0.4% solution of the resin in nitrobenzene and by possessing substantially complete solubility in aromatic hydrocarbons, by which is meant that at least 97% of the resin is completely soluble in the familiar benzenoid aromatic hydrocarbons such as benzene, toluene, and xylene. At weight concentrations of the resin up to and including 32%, solution viscosities are within a range which enables the compositions to be applied to surfaces by the usual means of application, such as direct roller coating. Polymeric materials containing only carbon, hydrogen, and chlorine having such chlorethylene units in which the chlorine content may be from 61% to 64% and which are within the above definition, provided, of course, that they possess the required viscosity and solubility characteristics, include certain interpolymers made from monomeric mixtures containing vinyl and vinylidene chloride only, or vinyl and vinylidene chloride together with polymerizable hydrocarbons or chlorinated hydrocarbons, such as styrene, dichlorostyrene, isobutylene and ethylene and mixtures of such interpolymers with each other or with other chlorine containing polymers such as polyvinyl chloride and polyvinylidene chloride which may result from the primary interpolymerization process. Polyvinyl chloride itself, and polyvinylidene chloride itself are, of course, not included, since the chlorine content of the first named polymer is below 61% and the chlorine content of pure polyvinylidene chloride is above 64%.

As mentioned previously, the aromatic hydrocarbon diluent not only serves the diluent function with respect to the dispersion resin but also acts as a solvent for the solution resin. This aromatic hydrocarbon solvent solubility of the vinyl chloride-vinylidene chloride solution resin permits the inclusion of a much larger percentage of solution resin in the organosol, and thereby a greater quantity of nonvolatiles in the organosol, while still maintaining a relatively low viscosity, than has heretofore been possible. This property of the organosols of the present invention enables them to be quickly and efficiently applied to flat metal sheets by the direct roller coating technique and to produce an easily fused, inert, and protective film, ridge free, with excellent smoothness, hardness, and gloss, a result unobtainable with prior art organosols.

The specific solution resin, in combination with the specific proportions and types of dispersants and diluents set forth above, also obviates the need for monomeric chemical plasticizers usually used in organosol compositions to obtain a continuous, cohesive film. In some unknown manner, all or part of the combination of solution resin, dispersant, and diluent performs the functions of the monomeric chemical plasticizers. By omitting the monomeric chemical plasticizer from the composition, the difficulties and disadvantages occasioned thereby, i.e., smoke evolution during fusing, lowered inertness and resistance of the film, are obviated. The solution resin imparts substantial cohesive strength to the final film and being polymeric, it is not leached out of the coating or appreciably attacked by strongly acid or alkaline fluids as are monomeric plasticizers. Further, due to the low volatility of the solution resin in comparison to monomeric plasticizers, the instant organosols containing the specific solution resin and no monomeric chemical

plasticizer evolve no obnoxious smoke during fusing of the dispersion resin.

The amount of the vinyl chloride interpolymer solution resin in the organosol must be in the range of from about 2% to 25%, and preferably about 10% by weight of the nonvolatile content. Quantities less than the specified minimum result in a final, dry coating having insufficient cohesive strength which tends to "mud-crack." Amounts of solution resin greater than the indicated maximum cause too great an increase in the viscosity of the fluid organosol composition; and overshadow the inert and resistant properties of the dispersion resin, giving the dry film more of the properties of the solution resin.

A polymeric plasticizer is included in the instant organosol to provide the final film with flexibility. The polymeric plasticizer is not to be confused with the monomeric chemical plasticizers generally used as dispersants in organosols. The polymeric plasticizer has little or no swelling or dispersing action on the dispersion resin. Although it is liquid at room temperature, it has very low volatility, and therefore does not distill or smoke during the fusing operation. Because it is polymeric, the plasticizer is much more resistant than the monomeric plasticizers to chemical attack by such materials as strong acids or bases.

The polymeric plasticizer I have found operable in the present invention is a soft, low molecular weight copolymer of a butadiene-1,3 hydrocarbon and an acrylic nitrile of the formula:



wherein R is selected from the class consisting of hydrogen, chlorine, and alkyl radicals. Such copolymer plasticizers are quite different in properties from butadiene acrylonitrile synthetic rubbers, which are of high molecular weight and of an elastic rubbery nature. The rubbery copolymers have average molecular weights considerably above 100,000, usually in the neighborhood of 150,000 or 175,000 or more; whereas the plasticizer copolymers have an average molecular weight of less than 85,000 and preferably below 65,000. Further, the elastomeric copolymers have a Mooney viscosity, i.e., a measure of softness and plasticity wherein the lower values represent greater softness and plasticity, of 50 or more; whereas the plasticizer copolymers exhibit a Mooney viscosity below 35.

The soft low molecular weight copolymers of this class found to be particularly effective in the practice of this invention are the copolymers of butadiene-1,3 or isoprene with acrylonitrile, chloroacrylonitrile, methacrylonitrile and ethacrylonitrile. Especially good results are obtained when the plasticizing material is made by the copolymerization under conditions adapted to produce a soft low molecular weight polymer of from 50 to 80 parts by weight of butadiene-1,3 and 20 to 50 parts by weight of acrylonitrile although copolymers from as little as 30 parts butadiene-1,3 and as much as 70 parts acrylonitrile may also be used. The best results are obtained with soft low molecular weight copolymers made by polymerizing in aqueous emulsion substantially 2 parts by weight of butadiene-1,3 and 1 part by weight of acrylonitrile. A polymeric plasticizer well suited for the practice of the instant invention and meeting the above specifications is marketed commercially under the name Hycar 1312.

The copolymer plasticizer is what is referred to in the art as a primary plasticizer. By this is meant that the copolymer may be used as the sole plasticizer in the organosol and still produce a final, dry film having the particular desired properties; or it may be used in combination with one or more polymeric, secondary plasticizers, the latter supplying some other desired property. Secondary plasticizers are not operable as the sole plasticizer in subject organosol.

The plasticizer used in the present invention, whether it is composed solely of the copolymer primary plasticizer

or of a combination of the primary plasticizer and a secondary plasticizer, must be compatible with both the dispersion resin and the solution resin and must have a low volatility even at the fusing or baking temperature of the organosol. The final, dry film must have sufficient flexibility to withstand the bending and forming operations performed on the metal substrate during its fabrication into a commercial item, such as an end for a metal can; but at the same time, the film must be sufficiently hard to resist abrasion during the forming operations and inert to provide chemical resistance. To accomplish these results, the total amount of plasticizer that may be present in the organosol, whether it be all primary or a combination of primary and secondary plasticizers, is in the range of from about 10% to 30%, and preferably about 20% by weight of the nonvolatiles. The ratio of primary to secondary plasticizer can be adjusted as desired according to the specific property sought. However, the amount of secondary plasticizer must be less than the amount of primary plasticizer, i.e., the weight ratio of primary to secondary plasticizer must be greater than 1 to 1, so that the properties of the primary plasticizer predominate.

The secondary plasticizers are also polymeric materials so as to be substantially non-fugitive by the action of heat and to be chemically inert. Examples of such secondary plasticizers are highly chlorinated paraffin waxes, epoxidized esters of a polyhydric alkanol and oleic or linoleic acid, particularly an epoxidized soybean oil polymer, and saturated, aliphatic polyesters. The epoxidized esters are described in United States Patent 2,485,160. The saturated, aliphatic polyesters are preferred as the secondary plasticizer, especially polyesters having a molecular weight of about 1,200 to 1,300.

In addition to the essential ingredients set forth hereinbefore, other ingredients commonly added to organosols may be incorporated as desired. For example, there may be added pigments such as titanium dioxide and/or carbon black, and/or heat stabilizers for the vinyl chloride resins such as blue lead. The amounts of these optional ingredients added to the organosol will depend upon the particular result desired, but the total weight thereof should be less than 30% and preferably less than 10% of the nonvolatiles.

The following example is for the purpose of illustration only and is not to be considered as limiting the invention. All parts are by weight.

A diluent-dispersant blend is formed by mixing 2.62 parts of a toluene-xylene mixture, 0.61 part diisobutyl ketone and 0.81 part diethylene glycol monobutyl ether. Into this blend is dissolved 0.15 part of the vinyl chloride-vinylidene chloride interpolymer solution resin having a total chlorine content of from 61 to 64%, which interpolymer has been described hereinbefore, 1.05 parts of the preferred butadiene-acrylonitrile copolymer primary plasticizer and 0.30 part of the saturated, aliphatic polyester secondary plasticizer having an average molecular weight of about 1200 to 1300. To this solution is added 0.23 part dibasic lead phosphite, 0.15 part blue lead, 0.15 part titanium dioxide, 0.075 part carbon black and 3.01 parts of the dispersion resin, i.e., 100% polyvinyl chloride having an intrinsic viscosity in cyclohexanone at 20° C. of 1.52. The resulting slurry is run into a pebble mill and ground, while maintaining the temperature below 90° F. until a 5 to 6 grind (Hegman grind gauge) fineness is obtained. Depending upon the size of the input particles, this grinding operation takes from 8 to 24 hours. The organosol is then ready for application to the desired surfaces and may be stored for future use.

The fluid organosol coating compositions of the present invention have a nonvolatile content of from about 45% to 65% and preferably about 55% by weight of the organosol, and a viscosity at room temperature, i.e., 70° to 80° F., of about from 210 to 560, and preferably about 75 from 315 to 420 centistokes. The amount of film form-

ing resins contained in the nonvolatiles is from about 70% to 80%, and preferably about 75% by weight of the nonvolatile. The relatively high percentage of nonvolatiles, including film forming resins, and low viscosity of the subject organosols permits the quick and efficient application of these organosols by the direct roller coating technique and the ready formation of smooth, ridge free, glossy inert and resistant protective coatings for sheet metal. Coatings deposited from the subject organosol have special utility as the interior protective lining for metal cans containing caustic liquids such as high pH detergents. The instant organosols are stable over long periods of time whereby little or no settling of the solid particles therein occur. Any false body resulting from long standing is easily overcome by a brief period of stirring.

This application is a continuation-in-part of my pending application, Serial No. 631,431, filed December 31, 1956, now U.S. Patent 2,918,445.

It is thought that the invention and many of its attendant advantages will be understood from the foregoing description and it will be apparent that various changes may be made in the matter of the ingredients, their identity, and their proportions without departing from the spirit and scope of the invention or sacrificing all of its material advantages, the form hereinbefore described being merely a preferred embodiment thereof.

I claim:

1. A fluid organosol coating composition containing about from 45% to 65% nonvolatile ingredients by weight of the total composition, the remainder of said composition comprising a volatile liquid dispersant and a volatile liquid diluent, said dispersant being selected from the group consisting of an aliphatic ketone and an aliphatic ether-alcohol and mixtures thereof and constituting about from 10% to 50% by weight of the volatile liquid constituents of said composition, said diluent comprising an aromatic hydrocarbon solvent and constituting about from 50% to 90% by weight of said liquid constituents, said nonvolatiles comprising by weight about from 50% to 80% of a vinyl chloride polymer in particulate form substantially insoluble in and uniformly dispersed in said dispersant and diluent and having an average molecular weight of at least 20,000 and a combined vinyl chloride content of at least 90% by weight of said polymer, about from 2% to 25% by weight of a vinyl chloride-vinylidene chloride interpolymer consisting of recurring chloroethylene units having from 1 to 2 chlorine atoms on only one of the ethylene carbons and a chlorine content of about 61% to 64% by weight dissolved in said dispersant and diluent, and about from 10% to 30% by weight of a polymeric plasticizer compatible with each of said dispersed polymer and said dissolved interpolymer in their solid state, said plasticizer

being a copolymer of a butadiene-1,3 and a monomer having the formula



wherein R is selected from the group consisting of hydrogen, chlorine and an alkyl radical and having an average molecular weight of not more than 85,000 and a Mooney viscosity of not more than 35, said composition having a viscosity of about from 210 to 560 centistokes at a temperature of from 70° F. to 80° F.

2. The organosol composition set forth in claim 1 having a nonvolatile content of about 55% by weight of said composition.

3. The organosol composition set forth in claim 1 wherein the volatile liquid dispersant constitutes about 36% by weight of the combined dispersant-diluent mixture.

4. The organosol composition set forth in claim 3 wherein the dispersant is composed of diisobutyl ketone and diethylene glycol monobutyl ether in a weight ratio of about 0.75/1.

5. The organosol composition set forth in claim 1 wherein the volatile liquid diluent is selected from the group consisting of benzene, toluene, xylene, and mixtures thereof.

6. The organosol composition set forth in claim 1 wherein said vinyl chloride polymer comprises about 66% by weight of the nonvolatiles.

7. The organosol composition set forth in claim 1 wherein said vinyl chloride-vinylidene chloride interpolymer comprises about 10% by weight of the nonvolatiles.

8. The organosol composition set forth in claim 1 wherein said vinyl chloride-vinylidene chloride interpolymer is soluble in said diluent.

9. The organosol composition set forth in claim 1 wherein said polymeric plasticizer comprises about 20% by weight of the nonvolatiles.

10. The organosol composition set forth in claim 1 having a viscosity of about 315 to 420 centistokes when measured at 80° F.

11. The organosol composition set forth in claim 1 wherein said polymeric plasticizer is a copolymer of butadiene-1,3 and acrylonitrile.

#### References Cited in the file of this patent

#### UNITED STATES PATENTS

|           |                |       |               |
|-----------|----------------|-------|---------------|
| 2,459,125 | Cheyney        | ----- | Jan. 11, 1949 |
| 2,520,959 | Powers         | ----- | Sept. 5, 1950 |
| 2,791,600 | Schwaegerle    | ----- | May 7, 1957   |
| 2,918,445 | Tarwid         | ----- | Dec. 22, 1959 |
| 2,941,974 | Reymann et al. | ----- | June 21, 1960 |
| 2,946,702 | Bach           | ----- | July 26, 1960 |